

Oct. 22, 1935.

D. M. BOOTHMAN

2,017,851

PRODUCING BRONZE POWDER PIGMENTS

Filed June 27, 1933



INVENTOR  
Dale M. Boothman  
ATTORNEY

## UNITED STATES PATENT OFFICE

2,017,851

## PRODUCING BRONZE POWDER PIGMENTS

Dale M. Boothman, Oakmont, Pa., assignor to  
Aluminum Company of America, Pittsburgh,  
Pa., a corporation of Pennsylvania

Application June 27, 1933, Serial No. 677,811

22 Claims. (Cl. 134—76)

This invention relates to the production of bronze powder pigments. It relates especially to the disintegration of metals, such as aluminum, into fine flakes adapted for use as bronze powder 5 pigments in powder form or in paste form. More specifically, the invention relates to an improved method of producing aluminum bronze powder and aluminum bronze powder paste, and to the improved intermediate and final products obtained in the practice of the said method.

In the past, metallic flake powders for use as pigments, of which aluminum bronze powder may be considered representative, have been produced almost exclusively by stamping operations. 15 These operations were frequently conducted in the presence of a lubricant, and were usually followed by a polishing treatment designed to impart brilliance and good leafing properties to the metal flakes. When processes of this nature are applied to aluminum, sheet or foil having a thickness of about 0.016 inch (about 26 gauge) or less 20 is shredded or cut into small pieces and put through a rough stamp mill or the like to reduce or disintegrate it into large, soft ductile flakes 25 which constitute an intermediate product called "shrode". This shrode is subjected to further stamping, whereby it is at least partially reduced to fine powder. The resulting product is screened or otherwise treated to separate the fine flakes 30 from any coarse material which may be present, and the fine material is then, in some instances, ready for the market. For most purposes, however, and especially when the powder is to be used as a pigment, a subsequent polishing treatment 35 is necessary in order to produce a powder having the desired characteristics. The polishing operation and both of the stamping operations are inherently slow and laborious, and therefore relatively costly. When it is desired to market the 40 bronze powder in paste form, the powder produced in a loose dry condition as described hereinabove must be mixed with the proper amount of a suitable vehicle until a paste of the desired consistency is obtained. This procedure is also slow 45 and laborious in many instances.

In my copending application, Serial No. 597- 901, filed March 10, 1932, I have described an im- 50 proved method of producing shrode, which con- sists of coating aluminum sheet, foil, or scrap with a suitable lubricating material and subject- 55 ing it to repeated rolling in a suitable rolling mill or series of mills until the desired reduction or disintegration has been effected. This pro- cedure greatly expedites the production of shrode and reduces its cost. I have also disclosed in the

said application that aluminum bronze powder can be produced by continuing the rolling of the shrode until the metal is disintegrated to a suitable fineness. Powder that is satisfactory for many purposes can be produced in this way, and my discovery of this fact is a valuable contribu- 10 tion to the art of bronze powder making. How- ever, powder produced by my previously disclosed process sometimes required polishing or other treatment to improve its appearance and its suit- 15 ability for certain applications. For example, I have found that when aluminum powder is pro- duced by rolling under conditions that result in the production of satisfactory shrode, there is sometimes encountered a tendency on the part of 20 the finer flakes or particles to roll up together into pellets or agglomerates, or to break up into granular pieces before they have been rolled to the required thinness, which reduces the desir- ability of the powdered product for use as a pig- 25 ment.

The main object of my present invention is to provide an improved process of preparing fine, polished metal flakes or powders, in which the difficulties and disadvantages encountered in pre- 25 vious processes are avoided or overcome. Fur- ther specific objects of my invention are to pro- vide an improved method of preparing aluminum bronze powder in paste, cake, or powder form; and to provide improved articles of commerce 30 prepared by the said method. My invention has for further objects the attainment of such other operative advantages and results as are found to obtain in the processes and products described and claimed hereinbelow.

My invention contemplates the production of bronze powder flakes by the disintegration of aluminum scrap, shrode, or analogous material by rolling in the presence of sufficient lubricat- 40 ing material to form a cake with the metal parti- cles. I have found that when the lubricant is present in the proper quantity, the thin flakes do not roll up into pellets when subjected to disinte- grating treatment in a rolling mill. Another ad- 45 vantage of my new method of disintegration is that the surfaces of the particles are polished sufficiently to make a separate and additional polishing operation unnecessary, even when pro- 50 ducing powder for use as a pigment. A further advantage is that when the lubricant is present in the proper quantity, the thin flakes do not roll up into pellets when subjected to disinte- 55 grating treatment in a rolling mill. Another ad- vantage of my new method of disintegration is that the surfaces of the particles are polished sufficiently to make a separate and additional polishing operation unnecessary, even when pro- 60 ducing powder for use as a pigment. A further advantage is that when the lubricant is present in the proper quantity, the thin flakes do not roll up into pellets when subjected to disinte- 65 grating treatment in a rolling mill. Another ad- vantage of my new method of disintegration is that the surfaces of the particles are polished sufficiently to make a separate and additional polishing operation unnecessary, even when pro- 70 ducing powder for use as a pigment. A further advantage is that when the lubricant is present in the proper quantity, the thin flakes do not roll up into pellets when subjected to disinte- 75 grating treatment in a rolling mill. Another ad- vantage of my new method of disintegration is that the surfaces of the particles are polished sufficiently to make a separate and additional polishing operation unnecessary, even when pro- 80 ducing powder for use as a pigment. A further advantage is that when the lubricant is present in the proper quantity, the thin flakes do not roll up into pellets when subjected to disinte- 85 grating treatment in a rolling mill. Another ad- vantage of my new method of disintegration is that the surfaces of the particles are polished sufficiently to make a separate and additional polishing operation unnecessary, even when pro- 90 ducing powder for use as a pigment. A further advantage is that when the lubricant is present in the proper quantity, the thin flakes do not roll up into pellets when subjected to disinte- 95 grating treatment in a rolling mill.

duct the disintegration that powder of extreme thinness as well as fineness is produced. This is one of the important features which distinguish my present "cake-forming" process from previous processes, as loose or substantially dry bronze powder flows readily and provides no "bite" for the rolls, and becomes increasingly difficult to roll as its fineness increases.

After the lubricant has been added to the shrode or other partially disintegrated metal and rolled or otherwise intimately mixed therewith to coat all the particles and hold them, without welding together, in the form of a cake, the consistency of the cake is not usually changed materially by subsequent disintegrating passes through the rolls; and when the disintegration is completed the product is in the form of a cake or thick batter. This represents a new and highly useful intermediate product in the bronze powder art, and may be readily converted into a high grade loose bronze powder, or into a bronze powder paste, as will be described in detail hereinbelow.

In carrying out my improved process, the choice of a proper lubricant is important. By the term "lubricant" as used herein, I mean a substance adapted to cover the surfaces of metallic particles with a thin layer of substantially uniform thickness, and to adhere to the particles with sufficient tenacity to prevent the welding together of individual flakes and preferably to prevent actual surface contact between them during rolling, but still having sufficient lubricating qualities—that is, viscosity, "oiliness", etc.—to permit the particles to move during rolling with sufficient freedom to impart a high polish to their surfaces. When bronze powders for use as paint pigments are to be produced, the aforesaid lubricants must also impart to the powder particles or flakes the ability to "leaf" well in paint vehicles, or an additional leafing agent or lubricant capable of imparting this property must be employed. Among the lubricating materials which are most suitable for my purpose are organic compounds of an unctuous nature, which are usually greases but may be oils. Of these, I generally prefer to use fatty acids, such as stearic, oleic, or ricinoleic acid or a mixture or combination thereof, but glycerides of the fatty acids, such as stearine, tallow or lard oil, are satisfactory and may be used if desired. The particular lubricant selected in any given instance may be determined by the qualities especially desired in the finished powder, such as whiteness, brilliance, or uniform opaqueness of the paint film.

In applying my process to the production of aluminum bronze powder flakes, I first prepare shrode by rolling aluminum stock as described in my prior application, or by other known methods of disintegration. To the shrode I add about one per cent (1%) by weight of a suitable lubricant, which is intimately mixed with the shrode before or during its reduction or disintegration. The amount of reduction required, and the consequently required duration of the disintegrating treatment or the number of passes between the rolls, vary according to the fineness of the shrode and the desired fineness of the final product. This may be readily determined for any given case, however, and in routine operation with known materials and known equipment, it is usually known in advance. When about 25% of the required reduction of the lubricated shrode has been completed by rolling in a suitable rolling mill or series of mills, it is usually desirable to add

another 1% of lubricant, after which the rolling treatment is continued until approximately 50% of the required reduction is completed. This may be when half of the required number of passes between the rolls has been completed, for example.

After about 50% of the reduction has been completed, and again when about 75% of the reduction has been completed, it is desirable to make further 1% additions of lubricant. This lubricant should preferably be adapted to impart good leafing properties to the powder produced, if the powder is to be used as pigment, whether or not the lubricant added during the first part of the reduction was adapted to act as a leafing agent. Thus I may use stearic acid, for example, throughout the rolling, as it is a satisfactory leafing agent and also a satisfactory lubricant, but I generally prefer to employ ricinoleic acid as the lubricant during the first part of the disintegration, because of its superior lubricating properties which result in a better surface-polishing action during the rolling, and permit rolling to the desired thinness without disintegration into granular particles. The additions of ricinoleic acid or other lubricants having a similar effect are accompanied or preferably followed by additions of stearic acid or some other suitable leafing agent. It is to be understood that my invention is not limited to the specific lubricants which I have mentioned as preferred, and also that the reduction or disintegration need not be carried out in four separate steps as above described. Instead the lubricant may be added continuously during the rolling treatment, and when more than one kind of lubricant is employed, the lubricants may be mixed and added to the metal particles together, or added alternately as the reduction proceeds.

The total quantity of lubricant employed may also be varied from the 4% of the weight of shrode or metal particles hereinabove specified. I have found, however, that substantially that amount of lubricant is generally preferable, especially when fine powder is to be produced. Quantities less than about 4% of the weight of the metal may not adequately cover the greatly extended surface of the final product as compared with surface of the starting material; and quantities greater than 4% are generally unnecessary and produce no additional advantages. Such larger quantities may usually be used, however, without detriment to the process or product, except that the metal content of the product may be unnecessarily reduced thereby. Sometimes, as when making coarse powders, quantities of lubricant as low as 2% of the weight of the metal give satisfactory results.

The thoroughness with which the lubricant is applied to and mixed with the shrode or particles produced therefrom has an important bearing on the quality of the powder produced, and I have found that it is desirable to spray the lubricant onto the particles or to knead it into them before the material enters the first roll pass, or between successive passes. In any case, it is essential that the metal surfaces be completely covered with lubricating material substantially throughout the rolling treatments which cause disintegration or reduction to the desired size. When this condition is maintained, and rolling is continued until substantially all of the metal has been disintegrated into flakes of suitable fineness for pigments or the like, the flakes have well

polished surfaces produced by the continued rubbing in the lubricant.

The pressure applied in the rolling mill is another important factor in determining the quality of the powdered product. Light pressure during the early stages of rolling facilitates the production of thin flakes, while heavy pressure tends to produce more granular material.

The polished flakes are discharged from the 10 rolling mill in the form of a thin cake held together by the lubricant. This cake is then treated to separate the flakes therefrom in the form of a loose, polished powder, or to produce a pigment paste, either of which may be readily 15 accomplished as will be described hereinbelow.

In order that my invention may be more readily understood, it will now be described with reference to the accompanying drawing, in which the single figure is a somewhat diagrammatic 20 elevational view, with parts in section, of one form of apparatus suitable for use in my process. In the drawing, a single pair of rolls 1 is shown, and the shrode 2 or like material to be disintegrated is passed and repassed through these rolls 25 until the desired reduction has been obtained, but it is obvious that a series of roll pairs or rolling mills may be employed if desired. The rolls 1 may have smooth surfaces, or one or both of them may be grooved, as described in my 30 aforementioned copending application, for example. The shrode is fed to the rolls from a storage hopper or analogous container 3 through a chute 5 or other suitable conveying means. Between the rolls 1 and the hopper 3 a mixing device 35 7 may be provided, for thoroughly mixing the metal particles with a lubricant which is supplied to the mixer from a tank or reservoir 8 as required. The mixer 7 may be of any desired type, such as a revolving drum with an internal agitator, or a covered pug mill, or a screw conveyor 40 which may replace the chute 5. The reservoir 8 may be heated, if desired.

The material discharged from the rolls passes through another chute or conveyor 10 adapted to 45 discharge into a suitable bin or hopper 12. A mixer 13 similar to the mixer 7 may be provided in this line for intimately mixing the metal particles with a lubricant or a leafing agent or the like, which is supplied from a reservoir 14, but either the mixer 7 or the mixer 13 can usually be 50 omitted. With the use of one or both mixers 1 can add the lubricant to the metal particles either continuously or in steps and thoroughly incorporate it in the resulting cake; or I can incorporate a lubricant in one mixer and another lubricant or leafing agent in the other.

When using only a single set of rolls 1 as shown 55 in the drawing, it is necessary to return the material first discharged by the rolls for further disintegration. The return of the material may be effected in any convenient manner, either manual or mechanical. When a mechanical return system is desired, an elevator 16 and belt conveyor 17 are suitable. The elevator may receive 60 material from the chute 10 or the bin 12, and may have the form of a bucket conveyor or a screw conveyor, for example. When the shrode has been suitably combined with lubricant and/or leafing agent and passed through the rolls until the desired disintegration has been effected, the 65 product in the form of a cake or thick mixture of fine, polished, flake-like particles of bronze powder 19 is allowed to accumulate in the bin 12 or some other suitable reservoir.

The further treatment of the cake 19 depends

on the form in which it is desired to obtain the final product, but in any event should be so conducted that the form and polish of the flakes is not impaired. When it is desired to produce a powder, it is necessary to apply a treatment to remove excess lubricant. This can be done conveniently and economically by mixing the cake with a suitable volatile solvent in a revolving drum 21 provided with a roll agitator 22 or other equivalent apparatus. The solvent is supplied 10 in controlled quantities from a reservoir 23, and is preferably an organic liquid such as ether, acetone, or toluol, which is capable of dissolving the lubricant without reacting with the powder particles. When solution of the lubricant is sub- 15 stantially complete, the fluid suspension is discharged from the drum 21 or other dissolving vessel into a tank 25 connected with an atomizing nozzle 26 provided with a compressed air connection 27, or the atomizer is connected di- 20 rectly to the drum 21, and the suspension is sprayed into a chamber 28, which is preferably heated. The solvent and a part of the lubricant volatilize and pass from the chamber 28 through a suitable condenser 30, where they are recov- 25 ered. Evaporation of the solvent leaves a coating of lubricant on the surfaces of the flakes, so that the leafing property and polish are retained, but the flakes deposit in the chamber in loose powder form and are suitable for use as a pig- 30 ment or for other purposes.

I have found that, in addition to removing excess lubricant from the cake by dissolving and then separating the powder from the solvent by evaporation as previously described, or otherwise, 35 treatments of a mechanical nature may be employed to separate the flakes from the cake. For example, the cake withdrawn from the hopper 12 may be gently tumbled in a revolving drum 21 with an inert solid granular material, such as 40 clean sand or particles of artificially prepared abrasive. The cake is easily broken up in this manner, and at least a portion of the excess lubricant is transferred to the surfaces of the larger, heavier particles of sand or the like. As a result 45 of the tumbling and the removal of the excess lubricant, the bronze powder particles are rapidly freed from the cake. The bronze powder is then readily separated from the sand or other relatively heavy material by an air separator 32 or 50 50 the like, operated in known manner, and is ready for use as pigment or otherwise. The sand can be freed from lubricant, as by washing in a solvent, and re-used if desired.

While my invention is advantageously used 55 in the production of loose bronze powder for pigments or the like, it has an especially advantageous application in the production of bronze powder pigment pastes. Such pastes are preferred to the loose powder for some purposes, as 60 is well known, and in the past the demand for a paste product has frequently been satisfied by preparing a loose powder and then mixing it with enough vehicle to form a paste of the desired consistency. This is often slow and laborious, 65 and therefore expensive, as the polished powder is not always wettable; and it is difficult to produce a product of uniformly high quality. By the process of my present invention, a pigment paste of high quality is uniformly and 70 economically produced. The cake 19 need only be agitated with mineral spirits or some analogous diluent and/or solvent for the lubricant to loosen the cake, whereupon a paste is readily formed. The complete operation can be carried 75

out very rapidly in the revolving drum 21 provided with a loose roll 22, or in a tank equipped with an agitator, or in other simple equipment, from which the paste is discharged in finished form. In the apparatus shown, the paste may be discharged from the drum 21 into the receiving vessel 25, from which it is withdrawn through an outlet 34 into shipping containers or the like.

Several modifications of this procedure are possible. For example, the paste may be formed by adding mineral spirits or other suitable thinner, solvent, or vehicle to the material recirculating through the rolls 1 when disintegration has been completed or substantially completed and the desired "cake" has been produced. This may be readily done by means of one of the mixers 7 and 13, to which the mineral spirits is supplied from the corresponding tank 8 or 14. Paste is then collected in the storage hopper 12, and the subsequent apparatus can be eliminated. If it is desired to remove some of the lubricant contained in the cake, this may be readily done by a slight modification of the method previously described. The mineral spirits or other solvent or diluent is then added to the cake in the revolving drum 21, or its equivalent, in a quantity more than sufficient to loosen the cake, and agitated to form a relatively thin slurry. This may be allowed to stand, whereupon the flakes settle, and the excess solvent containing some of the lubricant is decanted off, leaving a paste. The slurry may also be separated in a filter press or centrifuge, and similar methods may be employed for the recovery of loose powder by the solution method. While I prefer to employ mineral spirits as the solvent or thinner for the production of pigment pastes, solvent naphtha or turpentine or the like may also be used.

It will now be readily understood that my process offers many advantages over processes previously employed or proposed, in that the capacity of a properly operated rolling mill for disintegration or reduction of shrode and the like is much greater than the capacity of a stamp mill, for example; and in that the cake which I obtain as an intermediate product is a convenient material for the production of high grade polished bronze powders, and especially for the production of bronze powder pastes; and in other respects. While my invention has been described and illustrated with special reference to embodiments thereof which are now preferred, it is to be understood that certain other modifications and embodiments may be made without departing from the spirit of my invention, and within the scope of the appended claims.

I claim:

1. In a process of preparing aluminum bronze pigment, the disintegrating step comprising repeatedly rolling aluminum covered with a lubricant to form a cake of fine aluminum flakes held together by the lubricant.

2. In a process of preparing aluminum bronze pigment, the step comprising repeatedly rolling pieces of aluminum coated with a lubricating material adapted to prevent welding of pieces which overlap to disintegrate the aluminum into flakes and to form therefrom a thin cake held together by the lubricating material.

3. The process of preparing aluminum bronze pigment, which comprises repeatedly rolling aluminum material coated with a lubricant to

form fine flakes of aluminum bronze powder held together in the form of a cake by the lubricant, and separating the flakes from said cake.

4. In a process of preparing aluminum bronze pigment, the combination of steps comprising repeatedly rolling aluminum material coated with an organic lubricant to disintegrate the material into fine flakes of aluminum bronze powder held together in the form of a cake by the lubricant, and dissolving the lubricant to 10 separate the flakes from the cake.

5. The process of preparing aluminum bronze pigment, which comprises repeatedly rolling aluminum material coated with a lubricant to disintegrate the material into fine flakes of 15 aluminum bronze powder held together in the form of a cake by the lubricant, and mechanically separating the flakes from the cake.

6. The process of preparing aluminum bronze pigment, comprising repeatedly rolling aluminum 20 material coated with a lubricant to disintegrate the material into fine flakes of aluminum bronze powder held together in the form of a cake by the lubricant, and agitating the cake with an inert granular material to separate said flakes 25 therefrom.

7. The process of preparing aluminum bronze pigment, which comprises disintegrating aluminum material coated with a lubricating organic 30 material by repeated rolling, to form fine flakes of aluminum bronze powder held together in the form of a cake by the lubricant, and agitating the cake with a diluent to form aluminum bronze powder paste.

8. The process of preparing aluminum bronze pigment, which comprises repeatedly rolling thin 35 aluminum material with a lubricant to disintegrate the aluminum into fine flakes held together in the form of a cake by the said lubricant, agitating the cake with a solvent to dissolve at least a part of the lubricant and to loosen flakes from the cake, and separating loosened flakes of bronze powder from solvent containing dissolved lubricant.

9. The process of preparing aluminum bronze 40 powder, which comprises repeatedly rolling thin aluminum material with a lubricant to disintegrate the aluminum into fine flakes held together in the form of a cake by the said lubricant, agitating the cake with a solvent to dissolve at least 45 a part of the lubricant and to form a suspension of loosened flakes of bronze powder, spraying the suspension into a chamber to evaporate solvent, and collecting the loosened flakes of bronze powder. 50

10. The process of manufacturing aluminum bronze powder, comprising coating thin aluminum with a lubricant and disintegrating the aluminum by repeated rolling to form fine flakes of 60 aluminum bronze powder held together in the form of a cake by the lubricant, separating the flakes from the cake by agitating with solid inert particles heavier than the aluminum flakes and adapted to remove lubricant therefrom, and air-separating the bronze powder flakes from the inert particles. 65

11. The process of manufacturing aluminum bronze powder pastes, which comprises coating thin aluminum material with an unctuous organic lubricant and repeatedly rolling it to disintegrate the aluminum into fine flakes held together in the form of a cake by the lubricant, adding at least sufficient diluent to loosen the 70 75

cake, and subjecting the mixture to further rolling.

12. The process of manufacturing aluminum bronze powder pastes, which comprises coating thin aluminum material with an unctuous organic lubricant and repeatedly rolling it to disintegrate the aluminum into fine flakes held together in the form of a cake by the lubricant, adding a diluent capable of dissolving the lubricant, in a quantity more than sufficient to loosen the cake, agitating to dissolve lubricant, and withdrawing excess diluent with lubricant dissolved therein.

13. In a process of producing aluminum bronze pigment, the step comprising repeatedly rolling aluminum material with an organic lubricant to disintegrate the material into finely divided flakes of bronze powder with a finished polish and good leafing properties held together in the form of a cake by the lubricant.

14. In a process of producing aluminum bronze pigment, the combination of steps comprising mixing thin aluminum material with a lubricant, rolling to disintegrate the aluminum, adding more lubricant, and repeating the rolling and additions of lubricant to complete the disintegration and form fine polished flakes of bronze powder held together in the form of a cake by the lubricant.

30 15. In a process of producing aluminum bronze pigment, the combination of steps comprising mixing thin pieces of aluminum material with a lubricant adapted to prevent welding together of pieces of the aluminum under pressure, rolling the mixture to disintegrate the aluminum, adding a lubricant adapted to impart good leafing properties to the disintegrated aluminum, and continuing the rolling to form fine polished flakes of bronze powder with good leafing properties held together in the form of a cake by the lubricant.

40 16. In a process of producing aluminum bronze pigment, the step comprising rolling thin pieces of aluminum with about 4% by weight of a lubri-

cant to disintegrate the aluminum into fine flakes held together in the form of a cake by the lubricant.

17. In a process of producing aluminum bronze pigment, the step comprising rolling thin pieces of aluminum with about 4% by weight of a lubricant adapted to impart good leafing properties to the pigment to disintegrate the aluminum into fine flakes held together in the form of a cake by the lubricant.

10 18. In a process of producing aluminum bronze pigment, the step comprising rolling thin pieces of aluminum with about 4% by weight of a lubricant containing stearic acid to disintegrate the aluminum into fine flakes held together in the 15 form of a cake by the lubricant.

19. In a process of producing aluminum bronze pigment, the step comprising rolling thin pieces of aluminum with about 4% by weight of a lubricant containing ricinoleic acid to disintegrate 20 the aluminum into fine flakes held together in the form of a cake by the lubricant.

20. In a process of producing aluminum bronze pigment, the step comprising rolling thin pieces of aluminum with about 2% by weight of ricino- 25 leic acid, adding about 2% by weight of stearic acid, and continuing the rolling to disintegrate the aluminum into fine polished flakes having good leafing properties and held together in the form of a cake by the organic acids.

30 21. As a new product, fine polished flakes of aluminum bronze powder held together in the form of a cake by unctuous organic lubricating material.

22. As a new product, fine polished flakes of 35 aluminum bronze powder having good leafing properties and held together in the form of a cake by lubricating material comprising stearic acid and ricinoleic acid, said lubricating material being present in an amount equal to about 4% 40 of the weight of the powder.

DALE M. BOOTHMAN.